

## UNITED STATES PATENT OFFICE.

FREDERICK C. LANGENBERG, OF WATERTOWN, MASSACHUSETTS.

## ALLOY STEEL.

No Drawing.

Application filed January 24, 1927. Serial No. 163,297.

My invention relates to the provision of a new and improved alloy steel, and more particularly to an alloy steel containing manganese and molybdenum.

5 Heretofore, manganese steel alloys have been produced to which molybdenum was added with the result that the usual physical properties of the manganese steel were intensified. Steel alloys containing up to 10 about 3 per cent of manganese and as high as 1.25 per cent of molybdenum together with not more than about 0.80 per cent of carbon when properly heat treated have a high tensile strength and high elastic limit. 15 It is an object of the present invention to provide a steel alloy of this general type having improved physical properties, particularly, greater ductility and higher resistance to shock while maintaining a high 20 tensile strength and elastic limit.

It is a further object of the invention to provide a steel alloy containing manganese and molybdenum which may be molded to form sounder castings, with resulting improved physical properties, than is possible 25 with the ordinary manganese-molybdenum steel alloy.

As a result of extended investigations, I have found that the addition of zirconium 30 in small amounts to a manganese steel alloy, particularly one containing molybdenum, materially improves its physical properties. Higher ductility and greater resistance to shock is noticeable in particular in an 35 alloy of this type which contains a small amount of zirconium.

In general, the steel alloy of the invention should contain not more than about 0.90 to about 3 per cent of manganese and 40 not more than 1.25 per cent of molybdenum together with from about 0.10 to about 0.50 per cent zirconium and not more than about 0.80 per cent of carbon. The remainder of the alloy is composed of iron and slight 45 amounts of other elements incidental to the steel making process.

The alloy steel of the invention finds application in various fields, but I have found it particularly admirable for the manufacture 50 of castings for railway cars, such as bolsters and side frames. A suitable alloy steel composition for this purpose may contain from about 0.25 to about 0.45 of carbon and from about 1.25 to about 1.75 per cent of manganese together with from about 55 0.25 to about 0.50 per cent of molybdenum

and from about 0.15 to about 0.30 per cent of zirconium. Castings made from such an alloy steel composition, when properly heat treated, have very great resistance to shock 60 and at the same time are sufficiently strong and resistant to fatigue so that they can be made much lighter than similar castings heretofore produced.

If two manganese-molybdenum steel alloys are made of substantially the same composition except that one contains a small amount of zirconium, the one containing zirconium can be annealed or heat treated so as to give it the same elastic 65 limit and tensile strength possessed by the alloy not containing zirconium. When this is done it will be found that the alloy containing zirconium has much greater ductility and resistance to shock than the alloy which 70 does not contain this element. This is a most desirable feature when an alloy is to be subjected to dynamic or impact stresses.

On the other hand, a manganese-molybdenum alloy steel containing zirconium and which has substantially the same resistance 80 to impact as an alloy steel of substantially the same composition without the zirconium will have a higher elastic limit and tensile strength. In fact, if it is desired to have 85 a high elastic limit and tensile strength, the alloy of the invention may be heat treated to give these properties without seriously detracting from its resistance to impact. 90

## What I claim is:

1. An alloy steel containing substantial amounts of manganese and molybdenum but not more than about 3 per cent of manganese nor more than about 1.25 per cent of molybdenum together with from about 0.10 to about 0.50 per cent of zirconium. 95

2. An alloy steel containing from about 1.25 to about 1.75 per cent of manganese and from about 0.25 to about 0.50 per cent of molybdenum together with from about 0.15 to about 0.30 per cent of zirconium. 100

3. An alloy steel containing from about 1.25 to about 1.75 per cent of manganese and from about 0.25 to about 0.50 per cent of molybdenum together with from about 0.15 to about 0.30 per cent of zirconium and from about 0.25 to about 0.45 per cent of carbon. 105

In testimony whereof I affix my signature.

FREDERICK C. LANGENBERG.